

Patented Oct. 27, 1953

2,657,187

# UNITED STATES PATENT OFFICE

2,657,187

## DILUTE ALKALI DISPERSIBLE HOT MELT BOOKBINDING ADHESIVES

John Lloyd Evans, South River, and Dominic Donald Micucci, New Brunswick, N. J., assignors to E. I. du Pont de Nemours & Company, Wilmington, Del., a corporation of Delaware

No. Drawing. Application December 8, 1949,  
Serial No. 131,908.

7 Claims. (Cl. 260—30.8)

1

This invention relates to improvements in the art of binding books, catalogs, magazines and pamphlets with polymeric, organic, hot-melt-adhesives. More particularly, it relates to hot-melt, vinyl resin book-binding adhesives formulated to render them easily dispersible in aqueous dilute alkali solutions to permit waste paper disposal in a convenient manner.

In application Serial No. 593,099, filed May 10, 1945, having a common assignee with this invention is described a novel process of binding the page edges of books, magazines and similar articles of manufacture with solvent-free, hot-melt vinyl resin adhesive compositions which permits dispensing with the conventional step of stitching with cord or stapling associated with conventional glue binding. That hot-melt process has met with significant trade acceptance because of the permissible speed-up of the binding operations as a result of the quick setting of hot melt adhesives in comparison with the slow setting aqueous glues. Furthermore, a superior adhesively bound volume is obtained in comparison with the glue bound product reinforced with stitching or with crash which is subject to deterioration with age and by mold, moisture and loss of plasticity. Significant economy accompanied the adoption of the new process as a result of the increased rate of output, elimination of stitching or stapling steps and reduction in storage space normally required because of conventional practice of providing interrupted schedules for setting up the glue. Setting up of the glue is not represented by a precise schedule because atmospheric humidity conditions influence the rate at which the water is lost from the aqueous glue.

Although the hot melt process met with commercial success, the superior quality of the adhesives was detrimental in one particular respect indirectly effecting the economies of the process. The bookbinding operations involve considerable trimming and consequently scrap accumulation. It is not profitable to consume the scrap for its fuel value and therefore the trimmings are sold as scrap paper and eventually reused in some form of processed paper products. Scrap paper is graded according to established standards and priced accordingly. Scrap containing substantial foreign matter is saleable only at low prices.

Trimmings containing considerable vinyl resin adhesive are particularly objectionable as paper scrap because the adhesive is water insoluble and cannot be dispersed by conventional means used in de-inking operations and processes associated with paper manufacture and conversion. The undispersed adhesive particles, unless substantially removed, lead to spots or blemishes in the final paper product. These adhesive particles also clog the felting screens of the paper machine, thereby preventing proper felting of the pulp 50 to 55

2

slurry and consequently cause holes in final paper sheet. Adhesive particles are further deposited on the hot cylinder drying rolls where their adhesiveness may be sufficiently great to cause tearing of the felted paper web as it passes over the drying rolls.

As more and more hot-melt bookbinding adhesive is used, greater tonnage of catalogs, telephone directories, magazines and pocketbooks having the synthetic plastic adhesive incorporated therein will find its way into the scrap market and subsequently into the paper mills. Therefore, disposal of adhesive contaminated waste paper presents a serious problem.

It is an object of this invention to modify the bookbinding polymeric organic hot melt adhesives to remedy the above mentioned conditions in reference to waste paper disposal by rendering the adhesive dispersible in aqueous dilute alkali solutions normally used in conventional processing of paper scrap. Another object is to modify the composition of the polymeric adhesive chemically to provide susceptibility to dispersion in aqueous dilute alkali solution. A further object is to bind the edges of pages of books, catalogs and the like, without stitching or stapling using a vinyl acetate copolymer hot melt adhesive composition which is dispersible in aqueous dilute alkali. Still another object is to provide a book, catalog or similar article adhesively bound, without reinforcement with stitching or staples, by means of a vinyl acetate copolymer adhesive composition applied in hot melt condition, said adhesives being durable and resistant to water but which may be dispersed in aqueous dilute alkali to facilitate use of paper trimmings contaminated therewith and volumes subsequently disposed of as scrap paper.

These objects are accomplished by means of a hot melt adhesive composition which consists essentially of a copolymer of vinyl acetate and crotonic acid, preferably the polymerization product of 90 to 98 parts vinyl acetate and 10 to 2 parts of crotonic acid that is dispersible in aqueous dilute alkali solution, and methylated diaryl sulfone. Adhesive compositions formulated with these vinyl acetate-crotonic acid copolymers and methylated diaryl sulfone will deposit an adhesive film which has free carboxylic groups capable of salt formation with water soluble alkalies, such as sodium, potassium, and ammonium hydroxides, said salts promoting dispersibility and solubility in water.

In the preferred embodiment of this invention, the pages of a book, catalog or similar article are bound with a thermoplastic adhesive composition consisting essentially of a vinyl acetate-crotonic acid copolymer of the said proportions and  $\frac{1}{2}$  to 2 parts of a methylated diaryl sulfone having at least one methyl substituent on each

aryl group for each part of copolymer. A minor portion of a conventional compatible plasticizer, not more than 10% of the adhesive composition may be included in the composition for modification of flexibility. The term "liquefying" softener is used herein to describe softeners, which alter the properties of the vinyl acetate-crotonic acid copolymer from a thermoplastic resinous material having a gradual softening point to a composite blend having a sharply defined melting range as measured by the ball and ring method, said hot melt composition above its melting point rapidly becoming very liquid and capable of wetting and being adsorbed by the paper edges destined to become the backbone of the book.

The following examples are given by way of illustration only and no limitations are intended thereby except as indicated in the appended claims.

*Example 1*

The following components were charged into a polymerization kettle equipped with means for agitation, reflux and temperature control.

|                                       | Parts |
|---------------------------------------|-------|
| Dixylylsulfone                        | 220   |
| Vinyl acetate monomer                 | 300   |
| Crotonic acid                         | 14    |
| Polymerization initiator <sup>1</sup> | 0.9   |

<sup>1</sup>A suitable polymerization initiator is  $\alpha,\alpha$  azo bis (isobutyronitrile).

The mixture was constantly agitated at about 95 R. P. M. for the stirrer and the temperature raised to 70° C. and as the polymerization commenced the temperature increased gradually during about six hours to a temperature plateau at about 94° C. under slow reflux without altering the external source of heat, the temperature increase resulting from the conversion monomers to copolymer. 0.25 part of additional azonitrile polymerization initiator was charged into the kettle and polymerization continued under moderate to fast reflux for five additional hours during which time the temperature increased to a new plateau of about 105° C. Polymerization was then stopped by addition of 0.5 part of "Ionol" inhibitor, which is a Shell Chemical Company proprietary antioxidant. "Ionol" is described as one of the trialkyl-substituted "hindered" phenols having antioxidant properties, each of the said alkyl groups containing not more than 4 carbon atoms. More specifically, it is identified as 2,6 di-tertiary butyl 4 methyl phenol having a molecular weight of 220.3 and a melting point of 70° C. The unpolymerized vinyl acetate was removed by vacuum distillation at 50 mm. of mercury until the temperature of the melt reached 160° C. 86.8 parts of vinyl acetate were recovered as the distillate and the recovered product was 440 parts leaving an unaccountable loss of about 8 parts which apparently was vinyl acetate.

The product was calculated as having the following composition:

|                                       | Per cent |
|---------------------------------------|----------|
| Dixylyl sulfone                       | 50.0     |
| Vinyl acetate/crotonic acid copolymer | 49.9     |
| "Ionol" inhibitor                     | 0.1      |
|                                       | 100.0    |

The copolymer is estimated to consist of 93.6 parts vinyl acetate and 6.4 parts crotonic acid.

This hot melt adhesive was found to be thermally stable for 96 hours and longer at 160° C.

without loss of its dilute alkali dispersibility. By dilute aqueous alkali solutions is meant herein alkalinity of the order of the magnitude of .05% sodium hydroxide or its equivalent.

5 This hot melt adhesive used to bind books as shall be described later yielded an excellently bound volume having a tough, flexible backbone which was waterproof and resistant to deterioration with age and exposure to atmospheric conditions.

10 Rather than copolymerization in situ in the "liquefying" softener, the monomers may be copolymerized in orthodox solvents and subsequently compounded with the "liquefying" 15 softener and other desirable components to form the hot melt adhesive composition from which the solvent had been removed by distillation. The following example illustrates this practice.

*Example 2*

20 The following composition was charged into an agitated polymerization kettle.

|                                       | Parts by weight |
|---------------------------------------|-----------------|
| Toluene                               | 124             |
| 25 Vinyl acetate                      | 300             |
| Crotonic acid                         | 14              |
| Polymerization initiator <sup>1</sup> | 0.9             |

<sup>1</sup>A suitable polymerization initiator is azo bis (isobutyronitrile).

30 This mixture was heated to 70° C. and as polymerization proceeded, the temperature rose to a plateau at about 91° C. 0.25 additional part of initiator were charged into the kettle and polymerization continued until a plateau at about 35 98° C. was reached while under moderate reflux. 0.5 part of inhibitor was added to arrest the polymerization. 200 parts of molten dixylylsulfone were charged into the kettle and dispersed throughout the polymerized charge. The toluene and unpolymerized vinyl acetate were removed by distillation under vacuum at 50 mm. until the temperature reached 160° C. 176 parts of distillate and about 460 parts of adhesive were recovered. The adhesive was calculated to have 40 45 the following composition:

|                                       | Per cent |
|---------------------------------------|----------|
| Dixylylsulfone                        | 47.8     |
| Vinyl acetate/crotonic acid copolymer | 52.1     |
| Inhibitor                             | 0.1      |
|                                       | 100.0    |

50 The copolymer was estimated to contain about 5.6 parts of crotonic acid and 94.4 parts vinyl acetate.

55 This hot melt adhesive was equivalent to that of Example 1, exhibiting heat stability for 96 hours and longer at 160° C. without loss of its dispersibility in dilute alkali. Likewise applied in 60 the art of binding books with hot melt adhesives, it yielded an acceptably bound volume having the characteristics desirable for durable bindings and in addition, the adhesive contaminated trimmings and scrap thereof had full salvage 65 because the adhesive was adequately removed by alkali dispersibility by the orthodox operations.

70 By further experimentation it has been found that similar hot melt adhesive compositions in which the copolymer contained as little as 2% crotonic acid exhibit adequate dilute alkali dispersibility. The preferred content of crotonic acid is in the range of 2 to 10%, the balance being vinyl acetate. Still higher contents of 75 crotonic acid promote solubility in dilute alkali.

However, higher contents of this copolymerizable monomer leads to low molecular weight copolymers and exceptionally long polymerization cycles. The resulting low molecular weight copolymers are lacking in toughness, are soft and exhibit cold flow, properties which characterize the copolymer as inadequate for use in hot melt adhesives for binding books. Other fields of adhesive application may tolerate sacrifice in these properties and find utility for hot melt adhesives formulated with copolymers having a higher content than 10% of crotonic acid copolymerized therein. For example, such hot melts might be used for attachment of labels to glass and metal containers where it is desirable to subsequently remove the label by soaking in very dilute aqueous alkali solutions.

The foregoing examples show a two component hot-melt composition, that is, vinyl acetate-crotonic acid copolymer modified with a liquefying softener. It is obvious that such products may be modified with compatible orthodox ester plasticizers to alter the physical characteristics of the adhesive film. Generally the use of hot melt adhesives for the purpose of binding books limits the acceptable content of such plasticizers to 10% based on the total weight of non-volatile hot melt adhesive. Di(methyl Cello-solve) phthalate and triethyl citrate are particularly useful for plasticizing the vinyl acetate-crotonic acid copolymer adhesive. Tricresyl phosphate, diresyl carbitol, butyl phthalyl butyl glycolate, ortho-cresyl para-toluene sulfonate and polyethylene glycol di-2-ethyl hexoate may also be used. The latter plasticizer shows excellent compatibility with polyvinyl acetate, but its compatibility with the vinyl acetate-crotonic acid copolymer is more limited and in some instances it may not be used to the full extent of 10%.

It is obvious that the adhesive used for binding pages without the reinforcing action of staples or stitched thread to form the backbone of the volume must be characterized by greater toughness, flexibility and freedom from cold flow than adhesives used for other binding purposes, such as for attaching the cover to the said backbone. Consequently, for purposes of economy, the adhesive normally used in forming the backbone may be modified with low cost diluents when used as a cover adhesive. The following example is representative of a satisfactory cover adhesive which may be used either in combination with the hot melt bound backbone or alone to attach covers to stitched or stapled volumes.

*Example 3*

As in Example 2, the vinyl acetate and crotonic acid were copolymerized in toluene and the "liquefying" softener added to displace the solvent. The following ingredients were charged into the polymerization kettle with stirring:

Parts by weight

|                          |     |
|--------------------------|-----|
| Toluene                  | 124 |
| Vinyl acetate            | 300 |
| Crotonic acid            | 14  |
| Polymerization initiator | 0.9 |

Polymerization was carried out for about 7 hours while the temperature increased from 70° to 91° C. Then .25 part of additional polymerization initiator were charged into the kettle and the temperature increased from 91° C. to a plateau at 97° C. in about five hours. At this temperature, the polymerization was arrested by addition of .5 part of inhibitor ("Ionol"). 220 parts

of dixylyl sulfone were charged into the hot copolymer solution and distillation was commenced under 50 mm. vacuum to displace the toluene and remove the excess vinyl acetate. Distillation was stopped at 160° C., 200 grams of distillate having been recovered. To the solvent free hot melt adhesive remaining in the kettle were added 145 parts of dixylyl sulfone, 103.2 parts of Vinsol resin, 141 parts of Asbestine (a complex hydrated magnesium silicate of fibrous, crystalline structure) and 1.4 parts inhibitor for a final total charge of 841.1 parts.

This hot melt adhesive was found to be heat stable for about 96 hours at 160° C. and adequately retained its dispersibility in dilute alkali. The product used as an adhesive for attaching covers was found to be entirely satisfactory for the purpose. The use of the diluents, however, contributed brittleness and detracted from the toughness and flexibility inherent to the undiluted adhesive making it less desirable as a backbone adhesive.

The examples illustrate the invention using dixylyl sulfone as the liquefying softener. Other methylated diaryl monosulfones having at least one methyl substituent on each aryl group or mixtures thereof may be substituted in like amount. In addition to the dixylyl sulfone and its isomers, the various isomeric forms of ditolyl sulfone and xylyl tolyl sulfone are also particularly useful as the liquefying softener for the hot-melt adhesives of this invention.

Example 3 shows the use of resinous and mineral diluents. Still other diluents which are inert, non-volatile and heat stable for periods of 72 hours and longer in the presence of the hot melt composition at 160° C. may be used. Cotton flock, regenerated cellulose flake particles, glass fibers and the like which are generally characterized by dimensions of which the maximum on the average is about .12 inch and the ratio between length and diameter or thickness is in the range of 20-100 to 1, may also be used as diluents. Embedded in the applied adhesive, they exhibit reinforcing strength. Obviously due to matting effects, the amount of this diluent is limited. In the art of binding books and cover application, it is preferred that the content of this type of diluent does not exceed 7% based on the total adhesive composition.

The solvent used as a polymerization medium has an effect on the molecular weight of the polymer or copolymer. When tertiary butanol was used as solvent in place of toluene, a higher intrinsic viscosity product was obtained. However, in general, these copolymers have viscosities in the range of commercially low viscosity vinyl acetate polymers. The copolymerization can also be carried out in benzene or ethyl alcohol.

The nature of the polymerization initiator also affects the molecular weight of the copolymer. Peroxide initiators, such as lauroyl peroxide and benzoyl peroxide, and azonitrile initiators, such as  $\alpha',\alpha'$  azo-bis(isobutyronitrile) and  $\alpha,\alpha'$  azo-bis(alpha-gamma dimethyl) (valeronitrile) give copolymers having molecular weights which are satisfactory for hot melt adhesives and which are dispersible in dilute alkali. In general, any polymerization initiator which is satisfactory for the polymerization of vinyl acetate can be used for the copolymerization of vinyl acetate and crotonic acid.

It might be expected that introduction of carboxylic groups in the linear polymer contributes

alkali solubility and, therefore, an attempt was made to introduce such a group in a prepolymerized vinyl acetate resin by heating it with phthalic anhydride plus water.

*Example 4*

100 parts by weight of medium viscosity polyvinyl acetate were intimately mixed with 25 parts of phthalic anhydride and melted at a temperature of about 160° C. and with the kettle equipped with a reflux condenser, 10 parts of water were slowly added with continuous agitation of the charge. After 1 hour heating, distillation of the volatiles was commenced and heating continued for four hours. The distillate consisted of acetic acid and water, indicating that some ester interchange occurred between the vinyl acetate polymer and the phthalic acid. This modified polymer was found to be alkali soluble, at caustic soda concentrations of about 1.0% but not at the desired concentration of 0.1% and less, preferably about 0.05%. 50 parts of this polymer and 50 parts of a liquefying softener were melt-blended at about 160° C. to form a hot melt adhesive. The product was not heat stable as evidenced by gelation and charring. Crosslinking of the polycarboxylic phthalic acid by ester interchange in the vinyl acetate polymer presumably accounted for the gelation.

Attempts to overcome crosslinking by blocking one of the two carboxyl groups of the phthalic acid through the use of acid salts of phthalic acid failed to accomplish the desired objects. A copolymer of vinyl acetate and butyl hydrogen maleate also failed. Similarly, a difunctional reactant having both a carboxyl group and an inorganic acid reacting group, for example, metasulfobenzoic acid, failed by gelation. Furthermore, competitive ester interchange between a mixture of phthalic acid and a monocarboxylic fatty acid, such as stearic acid, with the vinyl acetate polymer failed to produce a modified vinyl ester polymer satisfactory for hot melt adhesive use.

Monofunctional acid reacting olefinic unsaturated materials which satisfactorily copolymerize with vinyl esters, particularly vinyl acetate were also tried. Acrylic acid and methacrylic acid polymerized in the presence of vinyl acetate yielded polymer compositions of non-uniform quality, apparently constituting mixtures of homopolymers and copolymers due to the significant difference in relative reactivities of the vinyl acetate and the acrylic and methacrylic acid in copolymerization.

It was indeed surprising to find that crotonic acid, isomeric with methacrylic acid, yielded uniform copolymers with vinyl acetate which are essential to the heat-stable, alkali-dispersible hot-melt adhesive particularly adaptable to the art of bookbinding.

The adhesives of the present invention may be used as other hot-melt adhesives in binding books. The basic design of a machine commercially used for binding books using glue is the bookbinding and covering machine described in the Bredenburg U. S. Patent 1,073,324, granted September 16, 1913. Numerous subsequent patents show modification in the machines and improved steps in the process of binding books involving such machines. Application Serial No. 593,099, filed May 10, 1945, describes modification of the process of binding books and similar articles by substitution of a solvent-free hot melt vinyl acetate adhesive composition for the glue and elimination of the steps of stitching or

stapling to reinforce the glue binding. Briefly, in commercial practice, the folded signatures subsequently to become pages of the bound volume are assembled between flat metal plates held together under pressure, the position of the gathered signatures being adjusted between the clamping plates to leave about  $\frac{1}{8}$  to  $\frac{1}{4}$  inch of page backbone edge exposed after the cutting operation has trimmed off the signature folds to reduce the signatures to a plurality of pages. The assembled clamped signatures are then passed through cutter to remove the said signature folds. The backbone now having a smooth uniform edge is subjected to roughers which serve the purpose of opening up the fibers at the edges of the pages to make them more receptive to the adhesive composition to provide better keying action by permitting the composition to penetrate into the interstices. Roughing may vary in degree and pattern to produce the desired keying action. The roughened edge is then freed of loose extraneous material by brushing, airblast or vacuum means. Following these preparatory steps, the hot melt adhesive is applied to the backbone edge by means of a conventional applicator roll consisting of a flat surfaced wheel revolving in and about  $\frac{1}{3}$  immersed in a hot melt adhesive, such as described in Examples 1 and 2, maintained at a temperature of about 160° C. An adjustable scraper-doctor blade or metering hot spinner removes the excess adhesive, leaving the desired thickness of film on the backbone. The adhesive application may be single stage or by multiple coats applied by subjecting the backbone to a series of adhesive applicators.

The application of a priming coat may precede the application of the principal hot melt adhesive. The primer is generally identical with the solvent-free, hot melt adhesive except it is cut with a volatile solvent which reduces the viscous hot melt to a very thin, penetrating liquid. The use of the primer necessitates provision of adequate means of substantially removing the volatile component of the applied primer prior to application of the hot melt. Obviously, since dilute alkali dispersibility is the object of the invention, it is pertinent that the deposited primer, like the principal adhesive, be characterized by that property.

As an alternative to priming the backbone of the book with a solution type primer, an aqueous dispersion of polyvinyl acetate containing a small percentage of polyvinyl alcohol as the dispersing and stabilizing agent may be used as a primer. Apparently the polyvinyl alcohol promotes dispersibility of the deposited primer in aqueous media, although a hot-melt adhesive formulated with vinyl acetate polymer is inadequately dispersible in dilute aqueous alkali solutions.

While the applied hot melt adhesive film is still in a substantial fluid condition an open mesh fabric or crash may be embedded therein to reinforce the backbone if such strengthening of the volume is desired. Finally the cover is attached following application of any of the solvent-free hot melt, heat-stable, alkali dispersible adhesives described herein. Example 3 which contains economical diluents is representative of a solvent-free hot melt adhesive entirely satisfactory for cover application. The covering machine often is separate from the main bookbinding machine which provides the means of converting the signatures to an uncovered volume having an adhesively bound backbone. Consequently, the covering operation using a hot melt adhesive may be employed in covering magazines, pocketbooks,

pamphlets, catalogs, etc. in which the signatures are held together with staples or stitched cord with or without the presence of conventional adhesives.

The trimming operations in the process of binding books, magazines and the like result in waste paper scrap contaminated with adhesive. When this adhesive is a conventional proteinaceous glue, the disintegration processes used by the paper converters in consuming the scrap cause the glue to disperse or dissolve, thereby providing a means of separation of substantially all of the adhesive to the extent that the ultimate product is unaffected by the small content of adhesive that may have been retained. When the adhesive is an orthodox resinous or elastomeric composition formulated with water insoluble polymers, the paper manufacturer using the waste paper encounters difficulty in using the scrap because the adhesive is not adequately and substantially dispersed and removed.

The waste paper and scrap contaminated with the adhesives of this invention formulated essentially with a copolymer consisting of the polymerization product of 90 to 98 parts vinyl acetate and 10 to 2 parts of crotonic acid and a compatible "liquefying" softener present no problem to the paper converter inasmuch as the adhesive is solubilized or dispersed in aqueous dilute alkali solution containing .05% sodium hydroxide, although dispersion in .01% caustic has been obtained by lengthening the contact time.

The trim or adhesive contaminated waste paper is generally consumed by paper mills in the manufacture of new paper. In some mills, as high as 80% of the furnish is waste paper with 20% being virgin pulp and the waste paper generally being magazine stock. Such operations involve repulping and de-inking steps which are described briefly to indicate that alkaline conditions adequate for dispersion of the adhesives of this invention exist in current practices. Repulping or defibering of the waste paper is carried out in a breaker beater or hydropulper where the waste paper is subject to mechanical action at a consistency of 5% paper and 95% water. During this mechanical operation, chemicals such as alkali, wetting agents, etc. are added for the purpose of de-inking the stock. De-inking is generally carried out at elevated temperatures in the range of 110° F. to about 180° F.

In a representative case the paper was repulped at a consistency of 4.5% and for de-inking the temperature was raised to 170° F., with a 6.0% sodium silicate and 1.4% sodium peroxide, on the basis of dry weight paper, being added as the de-inking chemicals. The processing cycle was three hours.

In another instance, 6000 pounds of dry paper were hydropulped at 3½% consistency followed by a 45 minute de-inking cycle at 180° F. in the presence of 200 pounds of soda ash and 100 pounds dry caustic soda.

In these instances, the alkalinity is in excess of the .05% suggested as the most suitable concentration for dispersing the hot melt adhesive.

Still another mill de-inked at 5% consistency at a temperature of 120° F. for a cycle ranging from 20 minutes to 2 hours using 1% caustic soda based on the dry paper. This caustic concentration is about .05%.

These mills which experienced serious difficulty in using waste paper contaminated with polyvinyl acetate to the extent that such type of scrap would not be purchased had no difficulty in using scrap contaminated with an equivalent adhesive in which the vinyl acetate-crotonic acid copolymer of this invention was substituted for polyvinyl acetate in the formulation.

A distinct advance in the art of bookbinding, particularly in the art of binding books, magazines, catalogs and the like with a solvent-free, hot melt polymeric resinous adhesive has been made by the use of adhesives comprises essentially of a copolymer consisting of the polymerization product of 90 to 98 parts by weight of vinyl acetate and 10 to 2 parts of crotonic acid and a "liquefying" softener, the latter being present preferably in the range of ½ to 2 parts for each part of copolymer. The use of the said hot melt adhesives characterized by dispersibility or solubility in aqueous dilute alkali at concentrations as low as .01% NaOH equivalent, preferably about .05% serves to eliminate a serious disposal problem in reference to use of waste paper contaminated with hot melt polymeric adhesive which heretofore was not dispersible during conventional waste paper processing. These advantages were economically accomplished without sacrifice in desirable characteristics of the adhesive, such as toughness, flexibility and freedom from cold flow.

It is apparent that many widely different embodiments of this invention may be made without departing from the spirit and scope thereof, and therefore, it is not intended to be limited except as indicated in the appended claims.

We claim:

1. A hot melt adhesive which is dispersible in a .05% aqueous alkali solution which comprises one part of a copolymer of from 90 to 98 parts of vinyl acetate and 10 to 2 parts of crotonic acid; and from ½ to 2 parts of a liquefying softener consisting essentially of a methylated diaryl sulfone having at least one but not more than two methyl substituents on each aryl group.
2. The composition of claim 1 which contains less than about 10% of a compatible solvent plasticizer.
3. The composition of claim 1 in which the liquefying softener is dixylyl sulfone.
4. The composition of claim 1 in which the liquefying softener is ditolyl sulfone.
5. The composition of claim 1 in which the liquefying softener is tolyl xylyl sulfone.
6. The composition of claim 1 in which the liquefying softener is a mixture of isomeric methylated diaryl sulfones.
7. The adhesive of claim 1 which contains a polymerization inhibitor.

JOHN LLOYD EVANS.

DOMINIC DONALD MICUCCI.

References Cited in the file of this patent

UNITED STATES PATENTS

| Number    | Name          | Date          |
|-----------|---------------|---------------|
| 1,659,401 | Kirschbraum   | Feb. 14, 1928 |
| 1,819,159 | Gale          | Aug. 18, 1931 |
| 2,127,400 | Gibbs         | Aug. 16, 1938 |
| 2,249,545 | Swan          | July 15, 1941 |
| 2,263,598 | Sarck et al.  | Nov. 25, 1941 |
| 2,310,725 | Widder et al. | Feb. 9, 1943  |
| 2,390,695 | Dean et al.   | Dec. 11, 1945 |